

1

2,880,053

**PROCESS OF TANNING HIDES WITH POLYMETHOXYALDEHYDE COMPOUNDS AND OPTIONALLY VEGETABLE TANNING**

Martin L. Fein, Riverside, N.J., and Edward M. Filachione, Philadelphia, Pa., assignors to the United States of America as represented by the Secretary of Agriculture

No Drawing. Application January 3, 1956  
Serial No. 557,217

3 Claims. (Cl. 8—94.21)

(Granted under Title 35, U. S. Code (1952), sec. 266)

A non-exclusive, irrevocable, royalty-free license in the invention herein described, throughout the world for all purposes of the United States Government, with power to grant sublicenses for such purposes, is hereby granted to the Government of the United States of America.

This invention relates to new reagents and new processes for tanning hides.

From time immemorial, man has largely depended on natural vegetable tannins for converting animal hides into leather. However, the supply of such materials is constantly diminishing and their cost increasing; consequently, great efforts have been made to develop suitable synthetic materials to replace the vegetable tannins. While many such synthetics have been used or suggested, none has been entirely satisfactory, either because of high cost or deficiencies in the properties of the leather produced thereby.

Accordingly, it is an object of this invention to provide new synthetic tanning agents that may be economically manufactured in any required amount and that react rapidly with hide substance to give a satisfactory tannage.

The process of the invention utilizes as tanning agents a class of long-chain aliphatic aldehydes called generically polymethoxyaldehydes and having the structure



wherein  $n$  has an average value of 2 to 20. Such aldehydes are readily obtainable by the hydrolysis of the corresponding acetals, particularly the methyl acetals having the formula



These acetals may be obtained by the condensation of methyl vinyl ether and methanol by any known process, such as, for instance, those described in U.S. Patents 2,165,962 and 2,487,525. Because of the great reactivity and consequent instability of the free aldehydes, we generally prefer to store them in the form of the acetal. The free aldehyde is then generated just prior to its use or it may actually be generated in situ during the tanning process.

Since the polymethoxyaldehydes are polymeric in na-

2

ture, it will readily be appreciated that the molecular weight and the value of  $n$  in the above formulas will be only an average figure for a given lot of material and that, in general, each lot will be a complex mixture, the individual molecules of which will have different chain lengths and values of  $n$ .

In the interest of brevity and simplicity, the average value of  $n$  in particular lots of material will be designated hereinafter by the appropriate numeral suffix; thus, 10 polymethoxyaldehyde-4 refers to a material in which the average value of  $n$  is 4. This we abbreviate as PMA-4.

By the term "hides" as used herein we mean any animal skin that is commonly tanned, such as cowhide, horsehide, calfskin, pigskin, sheepskin and goatskin, as well 15 as any such hide that has already been partially or completely tanned by a conventional tanning process. Any hide, as so defined, can be tanned by treatment with a polymethoxyaldehyde as shown hereinafter.

According to the invention, hides are tanned by immersion for a suitable time in a solution of polymethoxyaldehyde in water or a suitable organic solvent. No special preparation of the hide is necessary, the usual preparation for conventional tannage being entirely satisfactory. Likewise the amount and concentration of 25 tanning solution may be varied widely without detrimental effect. The affinity of the polymethoxyaldehydes for the hide substance is such that dilute solutions are substantially exhausted by the hides, yet the use of a large excess of tanning agent results in no loss because 30 the hide, when fully tanned, ceases to absorb the aldehyde.

The practice of the invention is illustrated by the following examples.

*Preparation of polymethoxyaldehydes.*—Polymethoxyacetals having average values of  $n$  in the above formulas 35 of 4, 9 and 14 were hydrolyzed to the aldehyde by stirring at room temperature with several times their volume of 1% aqueous hydrochloric acid until substantially all the acetal dissolved in the water layer. The small amount of insoluble material could be brought into solution by addition of a little alcohol or acetone, left in suspension or mechanically separated. The aqueous solution of aldehyde was adjusted to the desired pH by addition of alkaline reagents and/or buffers. If desired, the aldehyde may be similarly prepared in a suitable organic 45 solvent such as a lower aliphatic alcohol or ketone.

*Tanning with polymethoxyaldehydes.*—The aldehyde solutions prepared as described above were adjusted to the desired concentration, usually in the range 5 to 25%, though higher or lower concentrations could be used 50 without difficulty; the pH was adjusted by use of suitable buffers; salts such as sodium chloride or sulfate were added if desired and the hide, previously adjusted to the isoelectric point, was immersed in the solution. After being left at room temperature for various times, 55 with continuous agitation, samples of the hide were cut out, tested for shrink temperature ( $T_s$ ) and examined for leatherlike properties. Although the elevation in  $T_s$  was only moderately high, the samples, after being washed and dried were light colored and showed excellent leatherlike properties. A summary of the results of some typical experiments is shown in Table I.

Table I.—Tanning with polymethoxyaldehydes (PMA)

| Example   | Treatment |                           |                                      |           | Shrinkage Temp., °C., after— |        |        |        |
|-----------|-----------|---------------------------|--------------------------------------|-----------|------------------------------|--------|--------|--------|
|           | Aldehyde  | Buffer                    | Salt                                 | pH        | 1 day                        | 2 days | 3 days | 6 days |
| Cowhide:  |           |                           |                                      |           |                              |        |        |        |
| 1         | PMA-4     | Lactic acid, 5%           | NaCl, 5%                             | 3.3       | 60                           | 60     | 60     | 60     |
| 2         | PMA-4     | NaHCO <sub>3</sub> , 0.2M | None                                 | 7.1-7.6   | 74                           | 77     | 77     | 79     |
| 3         | PMA-4     | NaHCO <sub>3</sub> , 0.2M | NaCl, 4%                             | 7.1-7.5   | 74                           | 77     | 77     | 77     |
| 4         | PMA-4     | MgO, 0.4%                 | Na <sub>2</sub> SO <sub>4</sub> , 3% | 11.1-10.9 | 73                           | 74     | 74     | 74     |
| 5         | PMA-4     | MgO, 1%                   | NaCl, 3%                             | 10.6-10.4 | 72                           | 75     | 77     | 76     |
| 6         | PMA-9     | Lactic acid, 5%           | NaCl, 5%                             | 3.6-3.7   | 63                           | 61     | 61     | 70     |
| 7         | PMA-9     | NaHCO <sub>3</sub> , 0.2M | None                                 | 7.3-7.7   | 70                           | 72     | 72     | 74     |
| 8         | PMA-9     | NaHCO <sub>3</sub> , 0.2M | NaCl, 4%                             | 7.1-7.4   | 68                           | 70     | 70     | 72     |
| 9         | PMA-9     | MgO, 1%                   | NaCl, 3%                             | 10.2-10.1 | 68                           | 69     | 72     | 73     |
| 10        | PMA-14    | Lactic acid, 5%           | NaCl, 4%                             | 3.6-3.7   | 60                           | 60     | 60     | 60     |
| 11        | PMA-14    | NaHCO <sub>3</sub> , 0.2M | None                                 | 7.3-7.7   | 70                           | 73     | 73     | 74     |
| 12        | PMA-14    | NaHCO <sub>3</sub> , 0.2M | NaCl, 4%                             | 7.2-7.6   | 68                           | 70     | 70     | 71     |
| 13        | PMA-14    | MgO, 1%                   | NaCl, 3%                             | 10.5-10.3 | 67                           | 68     | 72     | 72     |
| Calfskin: |           |                           |                                      |           |                              |        |        |        |
| 14        | PMA-4     | Lactic acid, 5%           | NaCl, 5%                             | 3.3       | 58                           | 60     | 60     | 61     |
| 15        | PMA-4     | NaHCO <sub>3</sub> , 0.2M | None                                 | 7.3-7.9   | 73                           | 74     | 74     | 74     |
| 16        | PMA-4     | MgO, 0.4%                 | Na <sub>2</sub> SO <sub>4</sub> , 8% | 10.5-10.7 | 69                           | 71     | 71     | 71     |
| 17        | PMA-9     | NaHCO <sub>3</sub>        | None                                 | 7.6-8.0   | 68                           | 70     | 72     | 73     |
| 18        | PMA-14    | NaHCO <sub>3</sub>        | None                                 | 8.0-8.3   | 61                           | 69     | 71     | 73     |

Results similar to those shown in the table were obtained when other kinds of hide, such as horsehide, pigskin, sheepskin, goatskin or fur skins were used, or when the PMA was dissolved in alcohol, acetone or similar organic solvent instead of water. Likewise, PMA of higher or lower molecular weights, in the range of PMA-2 to PMA-20 gave equally satisfactory results. There is some advantage in using the lower molecular weight materials, such as PMA-2 to -10, in that they are more effective, pound for pound, they penetrate the hide faster and they are easier to prepare from the acetal.

Combination vegetable-aldehyde tannage in which vegetable tanned leather was retanned with PMA or in which PMA tanned leather was retanned with vegetable tannins gave products superior to those obtained by either tannage alone. They had higher shrink temperatures, were fuller and firmer and had better appearance. Furthermore retannage of the PMA tanned leather with vegetable tannins resulted in a much more rapid penetration by the latter agent.

We claim:

1. The process for tanning hides comprising impregnating the hides with an alkaline solution of a polymethoxyaldehyde having the formula



wherein  $n$  has an average value of 2 to 20 until the hides are tanned.

2. The process of claim 1 wherein the hide is first tanned with vegetable tannin and subsequently tanned with a polymethoxyaldehyde.

3. The process of claim 1 wherein the hide, after being tanned with a polymethoxyaldehyde, is subsequently tanned with vegetable tannin.

#### References Cited in the file of this patent

#### UNITED STATES PATENTS

618,722 Payne Jan. 31, 1899  
2,009,255 Friestedt July 23, 1935